

July 6, 1937.

C. B. GWYN, JR

2,086,221

CONTACT ASSEMBLY

Filed Dec. 10, 1934



INVENTOR  
Childress B. Gwyn, Jr.  
BY *John H. Gwyn*  
ATTORNEY

## UNITED STATES PATENT OFFICE

2,086,221

## CONTACT ASSEMBLY

Childress B. Gwyn, Jr., Indianapolis, Ind., assignor, by mesne assignments, to P. R. Mallory & Co. Inc., Indianapolis, Ind., a corporation of Delaware

Application December 10, 1934, Serial No. 756,733

7 Claims. (Cl. 200—166)

This invention relates to contact assemblies. An object of this invention is to produce an improved contact assembly.

5 A further object is to produce a more durable contact assembly having high electrical conductivity.

A still further object is to produce a contact assembly with a clean contact surface.

Other objects will be apparent from the following disclosure and drawing together with the appended claims.

According to one form of the invention, the above objects may be attained by the simultaneous application of pressure and electric current to the component parts of the contact assembly during assembling thereof whereby portions thereof are interfused. Furthermore, the component parts may be so shaped and prepared as to provide interlocking surfaces. Reservoir space may also be provided in the parts for any excess flow of metal developed during assembly.

The invention accordingly comprises the features of construction, combination of elements and arrangement of parts, referred to above or which will be further brought out and exemplified 25 in the disclosure hereinafter set forth, including the illustrations in the drawing, the scope of the invention being indicated in the appended claims.

For a fuller understanding of the nature and 30 objects of the invention as well as for specific fulfillment thereof, reference should be had to the following detailed description taken in connection with the accompanying drawing, in which:

35 Figure 1 is a top view of a contact member adapted for incorporation into a contact assembly.

Figure 2 is a side view of the contact member shown in Figure 1;

40 Figure 3 is a top view of a base or support member suitable for assembly with the contact member shown in Figures 1 and 2;

Figure 4 is a side view of the base member shown in Figure 3;

45 Figure 5 is a section on the line 5—5 of Figure 4;

Figure 6 is a diagrammatic illustration of the component parts of the contact assembly and part of the assembly machine during the assembling operation;

50 Figure 7 is a side view of a completed contact assembly; and

Figure 8 is a view, partly in section, of the completed assembly.

Like reference characters indicate like parts in the several figures of the drawing.

While a preferred embodiment of the invention will be described herein, it is contemplated that considerable variations may be made in the 5 method of procedure and the construction of parts without departing from the spirit of the invention.

Referring, now, more particularly to the drawing wherein one embodiment of the invention is 10 illustrated, a contact member or rivet 10 is shown in Figures 1 and 2 having a disc-shaped head 11 of non-refractory contact material, such as fine silver, for example, and a cylindrical shank 12 formed integrally therewith of the same material 15 or of a different metal, alloy or composition. Contact member 10 may be prepared by any standard and well known method such as by upsetting or heading.

A suitable base or support blank 13, for supporting contact member 10 after assembling is 20 shown more particularly in Figures 3 to 5. This comprises a portion 14 threaded or otherwise adapted to be secured in a suitable manner and position in electrical apparatus where the contact assembly is intended for use, and a recessed portion 15 adapted to receive contact member 10. Portion 14 may likewise be provided with a screw driver slot 30 or other means for adjusting the contact assembly in the electrical apparatus. 30 Portion 15 has a tapped or threaded hole or recess 16 therein of substantially the same diameter as shank 12, or of slightly smaller or larger diameter, as desired, and is intended to receive shank 12 upon assembly. Portion 15 is provided with 35 a substantially plane end surface 17 surrounding the mouth of hole 16 and adapted to serve as a seat for the underside of head 11 of the contact member 10.

A circular ridge 18 is formed on surface 17 and 40 encircles the mouth of hole 16. Ridge 18 provides for correct seating of contact member 10 on base member 13 and also provides for a reservoir space to receive any excess flow of metal during assembly and thereby prevent foreign 45 metals from reaching the upper contact surface.

Base member 13 may suitably be made of any desired metal or material commonly used in electrical parts such as brass or steel, for example. 50 The material is preferably one which is harder and has a higher melting point than the contact material.

The method of assembly may be as follows: Shank 12 of contact member 10 may be placed in

the mouth of hole 16 in base member 15 and axial pressure may be applied in any suitable manner such as by the press comprising plunger 19 and support 20 (Figure 6). Simultaneously with the 5 application of pressure an electric current of high density but of low voltage is passed through the assembly from the face of head 11 of the contact rivet 10 to the body of base member 13.

The current may be supplied in any desired 10 manner and may be either alternating or direct current. Alternating current may present some advantage over direct current since it lends itself to more accurate timing control by means of a thyratron control system. The current may 15 suitably be supplied, for example, as shown diagrammatically in Figure 6 by a step-down transformer 21 from the commercial alternating current supply. In this instance one low voltage terminal is connected to plunger 19 and the other 20 terminal to support 20. Current regulating equipment, shown as a variable resistance 22 is included in the circuit for controlling the current intensity and switching equipment shown 25 diagrammatically as contacts 23, is provided for starting and stopping the flow of current. A timing control 24 is preferably associated with the switching equipment for controlling the duration of the current flow. The above described electrical system is intended to be merely 30 illustrative of the general arrangement of parts and is in no sense intended to be limiting as to the type of equipment used or the mode of operation thereof. Thus the switching and control might be carried out on the high voltage side of 35 the transformer. The timing equipment might preferably comprise a thyratron control system.

The current is preferably so controlled in intensity and duration as to heat shank 12 to the 40 point of softening. Since the current density is greater in shank 12 than in the head 11 of the control rivet or the body of base member 13 these parts are not appreciably softened by the current. As the current softens shank 12 the pressure applied by plunger 19 forces the shank into 45 hole 16. The softened material of the shank flows into the thread grooves of hole 16, to form an interlocking structure.

After the shank 12 has been forced entirely 50 into the hole 16 so that contact head 11 seats squarely against ridge 18 on surface 17 the current is continued for an additional short period to bring about an interfusing or alloying of the material of the shank and of the threaded portion of hole 16, thereby forming an autogenous 55 weld between these parts. This current may also cause a fusing of ridge 18 into the bottom surface of contact 11 to further unite the contact head and backing member.

Should shank 12 inadvertently be made slightly 60 oversize or overlength so as to provide more than sufficient metal to fill hole 16 the excess metal may flow out of the hole and be received in the reservoir space formed by ridge 18 surrounding the hole. Thus the excess metal will 65 be kept from flowing to the upper contact surface. Normally, however, when there is no excess metal, ridge 18 is fused into the bottom surface of contact head 11 so closely that head 11 will seat directly against surface 17.

70 The completed contact assembly is shown in Figure 7 and illustrated in section in Figure 8.

As an example of the values of current, voltage, time and pressures required for making an assembly in actual practice, the following were 75 found to give satisfactory results:

On a contact assembly having a contact face of .125" diameter, of fine silver, a shank diameter of .078" and a commercial brass screw backing, using a 3-56 thread in the center, the instantaneous current, as read on an oscillograph, was 500 amperes A. C., the voltage applied to the assembly was 3.5 volts A. C. and the time the current was applied was 1 cycle A. C. or 1/60 second, governed by a thyratron control. The pressure applied to the surface of the contact 10 rivet 10 was 25 pounds.

Wide variations may be made, of course, in the practice of the invention both as to the form and structure of the component parts of the contact assembly, the type of assembling machinery used and the details of the assembly method. It is contemplated, for example, that the threading may be cut on the shank portion 12 instead of in hole 16, and that the hole and shank may be reversed in position, that is, the hole may be provided in the contact member and the shank in the backing member, if desired.

The present invention shows a marked improvement over previous contact assemblies and methods of making them. The method is well 25 adapted to practical production giving superior and more economical results than former methods of brazing, welding, mechanical staking or force fitting. When the relatively simple operation described above is completed there is little 30 or no further processing required beyond inspection.

The adjacent surfaces of the contact member and the base member are united by an autogenous 35 weld of low resistance. The weld prevents the occurrence of electrolytic corrosion or "battery action" between the surfaces of the two metals.

Since no lower melting brazing or welding materials are used, there is little danger of the 40 creeping of foreign materials to the contact surface. Furthermore, any excess metal flow developed during production will be held in the reservoir space and prevented from reaching the 45 contact surface.

The contact assembly parts are both welded together and interlocked rendering impossible 50 any loosening after repeated mechanical hammering or vibration or repeated expansion and contraction due to variations in temperature. The interlocking and welding arrangement likewise makes possible a shorter shank length than 55 with purely mechanical staking methods.

While the present invention, as to its objects and advantages, has been carefully described 55 herein as carried out in a specific embodiment thereof, I do not desire to be limited thereby but intend to cover the invention broadly within the spirit and scope of the appended claims.

I claim:

1. A contact support blank having a recessed portion for receiving a projection on a contact part, said recessed portion having formations for interlocking with said projection and having a reservoir for receiving excess metal.

2. A contact support blank having a hole in one of its surfaces for receiving a projecting shank of a contact part and a continuous ridge on said surface encircling the mouth of said hole.

3. A contact assembly comprising a contact part and a supporting part, one of said parts having a shank portion and the other of said parts having a recessed portion receiving said shank portion, one of said portions being thread- 75

ed, and an interfused junction between said shank portion and said recessed portion.

4. A contact assembly comprising a silver contact part and a base metal supporting part, one of said parts having a shank portion and the other of said parts having a recessed portion receiving said shank portion, one of said portions being threaded, and an interfused junction between said shank portion and said recessed portion.

5. A contact backing blank having a substantially plane face and a depression in said face, a circular disconformity in said surface surrounding said depression and spaced therefrom, said disconformity comprising a deviation of the surface from the plane of said face whereby said disconformity is adapted to stop the flow of molten contact metal outward from said depression.

6. A contact backing blank of steel having a substantially plane face and a depression in said

face, a circular disconformity in said surface surrounding said depression and spaced therefrom, said disconformity comprising a deviation of the surface from the plane of said face whereby said disconformity is adapted to stop the flow of molten contact metal outward from said depression.

7. A contact assembly comprising a steel backing member and a silver contact member fused thereto, the interface between said backing and contact members being characterized by a depression in said steel backing into which said silver extends, a substantially flat interface area surrounding said depression and a flow-restricting disconformity in said interface surrounding said flat area, said disconformity comprising a deviation of the interface from the plane of said flat area.

CHILDRESS B. GWYN, JR. 20